

June 29, 1948.

L. D. JORDAIN

2,444,047

## PROCESS OF PREPARING PAPER PULP FROM MARSH REEDS

Filed Nov. 8, 1946

2 Sheets-Sheet 1



Inventor:  
By: Louis D. Jordain  
Wallace and Cannon  
Attorneys

June 29, 1948.

L. D. JORDAIN

2,444,047

PROCESS OF PREPARING PAPER PULP FROM MARSH REEDS

Filed Nov. 8, 1946

2 Sheets-Sheet 2

Fig. 3.



Fig. 4.



Fig. 5.



Inventor:  
By Louis D. Jordain  
Wallace and Cannon  
Attorneys

## UNITED STATES PATENT OFFICE

2,444,047

PROCESS OF PREPARING PAPER PULP  
FROM MARSH REEDS

Louis D. Jordain, Princeton, Ill., assignor of one-third to Arthur I. Fleming, Princeton, Ill., and one-third to Howard E. Wagner, New York, N. Y.

Application November 8, 1946, Serial No. 708,659

6 Claims. (Cl. 92—17)

1

This invention relates to a process for making paper pulp from so-called marshland rushes or marsh grasses or reeds and like coarse grassy cellulose-bearing plants.

I am aware that attempts have been made heretofore to manufacture paper pulp from so-called marshland rushes or marsh grasses or reeds and the like but, insofar as I am aware, none of these processes has met with any commercial success.

In the development of the present invention I have found that in order to manufacture paper pulp successfully from so-called marshland rushes or marsh grasses or reeds or like coarse grassy cellulose-bearing plants it is essential that the various steps employed be carefully controlled and interrelated as in the process of the present invention and that the combination of steps employed in the new process is effective in successfully manufacturing paper pulp from such normally waste materials.

Accordingly, an object of the present invention is to provide a novel and efficient process for making paper pulp from so-called marshland rushes or marsh grasses or reeds and like coarse grassy cellulose-bearing plants.

Other and further objects of the present invention will be apparent from the following description and claims and by reference to the accompanying drawings.

In the drawings:

Fig. 1 is a view, largely diagrammatic but partly in vertical section, partially illustrating a typical flow diagram and a typical apparatus which may be employed in practicing the new process;

Fig. 2 is a view, largely diagrammatic, but partly in section, further illustrating a typical apparatus which may be employed in the practice of the process of the present invention and in the treatment of the paper pulp mat after the same has been discharged from the right hand end of the apparatus shown in Fig. 1;

Fig. 3 is an enlarged sectional view of the interfitting pressure dehydrating rollers which are shown adjacent the right hand end of Fig. 1 and which cooperate to express most of the liquid from the pulp mat at one step in the new process;

Fig. 4 is a central vertical sectional view on line 4—4 in Fig. 3; and

Fig. 5 is a view on line 5—5 in Fig. 3 partly in section and partly in elevation.

A suitable apparatus which may be employed in the practice of the new process of the present invention is illustrated largely diagrammatically in the drawings and is therein generally indicated at 10, and includes a plurality of tanks or receptacles 11, 12, 13, 14, 15, 16 and 17, which may be arranged in end to end relationship, and a dryer unit 18 (Fig. 2) which is arranged at the delivery or outlet end of the tank or receptacle 17. Thus

2

it will be seen that in the practice of the present invention all of the parts of the apparatus illustrated largely diagrammatically in Figs. 1 and 2 are arranged in end to end relationship but because of limitations of space the parts have been shown divided in Figs. 1 and 2 of the drawings.

The apparatus diagrammatically shown in the drawings and which may be used in the practice of the process of the present invention includes

10 a pair of rotatable pressure rollers 19 which rotatably mounted on suitable horizontally extending supporting shafts 21 which are rotatably mounted one above the other at one end of the tank 11, and a second pair of rotatable pressure rollers 20 which are rotatably mounted upon suitable horizontal shafts 21 which are rotatably mounted one above the other adjacent the other end of the tank 11 and in spaced relationship to the pressure rollers 19. A storage and discharge hopper 22 is mounted above the tank 11 and has a lower end portion providing a discharge outlet 23 which is arranged between the upper pressure rollers 19 and 20 above the tank 11 and is adapted to discharge material from the body of the storage hopper 22 between the pressure rollers 19 and 20 into the tank 11. This storage and discharge hopper 22 is adapted to contain and hold pulverized quick lime.

The apparatus 10 also includes an endless conveyor or belt 25 which is arranged in and is adapted to convey material through the tank 12. This endless conveyor or belt 25 works around a suitable guide roller 26 which is rotatably mounted adjacent the bottom of the tank 12 at one end thereof and the belt or conveyor 25 also works around a drive roller 27 which is journaled in a suitable support above the tank 12 at the opposite end thereof from the end at which the roller 26 is arranged.

40 A third pair of pressure rollers 28 are rotatably mounted on suitable horizontally extending shafts 29 which are mounted one above the other and above the tank 13 adjacent one end thereof.

A fourth pair of pressure rollers 30 are rotatably mounted on suitable mounting shafts 31 which are arranged one above the other above the tank 13 in spaced relationship to the pressure rollers 28. A storage and discharge hopper 32 is mounted above the tank 13 and has a lower end portion providing a discharge outlet 33 disposed between the upper pressure rollers 28 and 30 and adapted to discharge the contents of the hopper 32 into the tank 13.

An endless conveyor or belt 34 is arranged in 55 the tank 14. This endless conveyor or belt 34 works around a guide roller 35 which is rotatably mounted in the lower end portion of the tank 14 adjacent one end thereof. The endless conveyor or belt 34 also works around a drive roller 36 which is rotatably mounted above the tank 14 and

at the opposite end thereof from the end at which the guide roller 35 is arranged.

A pair of interfitting or intermeshing grooved pressure and dehydrating rollers 37 are rotatably mounted on suitable horizontally extending supporting shafts 38 which are arranged one above the other at one end of the tank 15 and a second set of grooved pressure and dehydrating rollers 39 are rotatably mounted upon suitable horizontal supporting shafts 40 which are arranged one above the other at the other end of the tank 15 and in spaced relationship to the pressure and dehydrating rollers 37. As shown in Figs. 3, 4 and 5, of the drawings, each of the pressure and dehydrating rollers 37 and 39 is provided on its peripheral surface with alternately arranged horizontally and axially extending ridges or teeth 50 and horizontally and axially extending grooves or recesses 51. As shown in Figs. 1, 3, 4 and 5 the ridges or teeth in one of the rollers 37 are adapted to engage in the grooves or recesses 51 in the other roller 37 and the ridges or teeth in one of the rollers 39 are adapted to engage in the grooves or recesses 51 in the other roller 39.

An endless conveyor or belt 41 is arranged in the tank 16. This endless conveyor or belt 41 works around a suitable roller 42 which is rotatably mounted in the lower end portion of the tank 16 adjacent one end thereof. The endless conveyor or belt 41 also works around a suitable drive roller 43 which is rotatably mounted above the tank 16 adjacent the end thereof which is opposite the end at which the guide roller 42 is mounted.

A pair of pressure rollers 52 are rotatably mounted upon suitable horizontally extending supporting shafts 53 and are arranged one above the other at one end of the tank 17. A second set of pressure rollers 54 are rotatably mounted upon suitable horizontally extending shafts 55 which are arranged one above the other at the other end of the tank 17 and in spaced relationship with the pressure rollers 52.

The drying unit 18 includes an upper endless conveyor or belt 44 which works around suitable drive rollers 46 and around suitable guide rollers 45. The drying unit 18 also includes a second and lower endless conveyor or belt 47 which works around suitable guide rollers 48 and around suitable drive rollers 49.

The mountings and supports and the drawing mechanisms for the various rollers and other parts of the apparatus which is shown largely diagrammatically in Figs. 1 to 5, inclusive, of the drawings, may be of any suitable design and construction.

In the use of the process of the present invention the paper pulp stock in the form of so-called marshland rushes or marsh reeds or like coarse grassy cellulose bearing materials are fed by means of a suitable conveyor (not shown) along the flow line 24 between the first pair of pressure rollers 19 which flatten and crush the reeds and extract therefrom part of the natural fluid content or juices borne by such reeds and which drains therefrom into the tank 11. As the stock passes out of the first pair of pressure rollers 19 and into and between the second pair of pressure rollers 20 pulverized quick lime is discharged from the lower end or outlet portion 23 of the hopper 22 onto the stock. For this purpose I have found that a suitable quantity of pulverized quicklime is one pound of the pulverized quicklime to approximately one hundred pounds of the stock. However, the percentage may be varied

depending upon variable factors, including the age of the reeds, and their maturity, and may be increased up to ten pounds of pulverized quicklime for each one hundred pounds of stock if the marsh reeds or like stock are relatively mature, dry and coarse.

The stock thus mixed with pulverized quicklime from the hopper 22 then passes into and between the second pair of pressure rollers 20 which exert a further crushing action on the stock and also press the quicklime into the stock.

The thus treated stock then passes along the flow line 24 into the tank 12 which contains warm water which acts upon the quicklime to slacken the same. As the stock enters the tank 12 it is discharged onto the endless conveyor or belt 28 and as it passes through the tank 12 it is borne up the endless conveyor or belt 25 and during this operation the slackened lime acts upon the pith, chlorophyl and natural waxes which bind the plant fibers together to separate these materials from the natural cellulose of the reeds or like stock. At this stage in the process the stock acquires the form of a loose mat and is discharged from the endless conveyor or belt 25 into and between another and third pair of pressure rollers 28 which serve to expel the bulk of the thus loosened pith, chlorophyl, and natural waxes and other residuary material from the plant fibers, these materials being thereupon drained into the tank or receptacle 13.

As the mat emerges from the pressure rollers 28 a bleaching mixture of pulverized quicklime, common salt and powdered sulphur is discharged from the lower end or outlet 33 of the hopper 32 onto the mat. For this purpose I have found that a bleaching mixture containing ninety-five per cent, by weight, of quicklime, two per cent of common salt or sodium chloride and three per cent of powdered sulphur is well suited for its intended purpose which is primarily to bleach the stock and secondarily to expel residual materials from the plant fibers in the mat.

The mat with the bleaching mixture thus mixed therewith is then fed between a fourth pair of pressure rollers 30 which further pulverize the bleaching mixture and press it into intimate association with the mat itself as the mat passes between the pressure rollers 30.

The mat is then discharged along the flow line 24 into the tank 14 and onto an endless conveyor or belt 34.

The tank 14 is adapted to contain hot water and as the mat passes through the tank 14 on the endless conveyor or belt 34 the hot water in the tank 14 operates on the bleaching mixture of pulverized quicklime, common salt and powdered sulphur to effect a chemical reaction between these materials to form a bleaching solution probably according to the following general reaction:



The mixture in the tank 14 while functioning primarily as a bleaching solution also serves to defiber the stock as the mat passes through the tank 14.

As the mat leaves the tank 14, by way of the endless conveyor or belt 34, it passes along the flow line 24 between the interfitting pressure and dehydrating rollers 37 and thence between the interfitting pressure and dehydrating rollers 39. As the mat passes through these pairs of pressure and dehydrating rollers 37 and 39 it is forced by the ridge-like teeth 50 thereof into the grooves

or recesses 51 formed in the peripheral surfaces of these rollers and most of the fluid or liquid content of the mat is thus expelled therefrom and drained into the tank 15.

As the mat emerges from the pressure and dehydrating rollers 39 it follows the flow line 24 into the tank 16 wherein it is discharged onto an endless conveyor or belt 41 and as it passes through the tank 16 on the endless conveyor or belt 41 it is subjected to the action of clear cold water in the tank 16. This action washes out most of the impurities in the mat so that the mat emerges from the tank 16 on the endless conveyor or belt 41 as a substantially clean paper pulp mat.

The thus treated paper pulp mat then follows the flow line 24, from the right hand end of the apparatus shown in Fig. 1 into the left hand end of the apparatus shown in Fig. 2, and is directed between the pair of pressure rollers 52 and thence between a second pair of pressure rollers 55 which press substantially all of the water out of the pulp mat and convert the same into a substantially homogeneous endless paper pulp mat or sheet. The liquid expressed from the mat during this operation flows into the tank 17.

The paper pulp mat thus formed then passes along the flow line 24 into the drying apparatus 18 and onto the lower endless belt 47 and between the latter and the upper endless belt 44 by which the mat is conducted through the drying apparatus 18 and is thus dried.

The thus prepared paper pulp emerges from the drying apparatus 18 as a substantially homogeneous paper pulp mat and is then ready for a baling or reeling whereupon it may be delivered to a paper mill for further processing or use.

The waste products collected in the tank 11 may be processed into suitable by-products such, for example, as commercial ethyl alcohol and other materials, and the waste by-products collected in the tank 13 may be used for fertilizer. Likewise, the waste material collected in the tank 15 may be used as a fertilizer which is especially adapted for use with citrus trees.

It will thus be seen from the foregoing description, considered in conjunction with the accompanying drawings, that the present invention provides a novel process for preparing a paper pulp mat from natural so-called marshland rushes or marsh reeds or like coarse grassy cellulose-bearing natural plants which are ordinarily waste materials and available in large quantities. Hence the present invention has the advantages and desirable characteristics and accomplishes its intended objects including those hereinbefore pointed out and others which are inherent in the invention.

I claim:

1. A process of preparing paper pulp mat from marsh reeds which comprises the steps of crushing the said marsh reeds, discharging pulverized quicklime onto the crushed marsh reed stock, further crushing the marsh reed stock having the pulverized quicklime intermixed therewith, passing the thus crushed marsh reed stock having the said quicklime mixed therewith through water to slacken the said quicklime and to convert the said crushed marsh reed stock into the form of a loose mat, further crushing the said loose mat thus formed, bleaching the said mat and converting it into the form of a substantially homogeneous paper pulp mat, expressing the

liquid content from the said mat after the bleaching operation, then washing the mat in water, expressing the bulk of the water from the thus washed mat, and then drying the mat.

5 2. A process of preparing paper pulp mat from marsh reeds as defined in claim 1 in which the operation of bleaching the mat is effected by discharging onto the moving mat a mixture of pulverized quicklime, sodium chloride and powdered sulphur and then passing the mat with the said bleaching mixture thereon through warm water.

10 3. A process of preparing paper pulp mat from marsh reeds as defined in claim 1 in which the operation of bleaching the mat is effected by discharging onto the moving mat a mixture consisting of approximately ninety-five (95) per cent of pulverized quicklime, two (2) per cent of sodium chloride, and three (3) per cent of powdered sulphur, by weight, and then passing the mat having the said bleaching mixture intermixed therewith through warm water.

15 4. A process of preparing paper pulp mat from marsh reeds as defined in claim 1 in which the said quicklime is discharged onto the initially crushed marsh reed stock in a ratio of about one (1) pound of quicklime to about one hundred (100) pounds of the said initially crushed marsh reed stock, by weight.

20 5. A process of preparing paper pulp mat from marsh reeds as defined in claim 1 in which the said quicklime is discharged onto the initially crushed marsh reed stock in a ratio of about one (1) pound of quicklime to about one hundred (100) pounds of the said initially crushed marsh reed stock, by weight, in which the operation of bleaching the mat is effected by discharging onto the moving mat a mixture of pulverized quicklime, sodium chloride and powdered sulphur and then passing the mat with the said bleaching mixture thereon through warm water.

25 6. A process of preparing paper pulp mat from marsh reeds as defined in claim 1 in which the said quicklime is discharged onto the initially crushed marsh reed stock in a ratio of about one (1) pound of quicklime to about one hundred (100) pounds of the said initially crushed marsh reed stock, by weight, in which the operation of bleaching the mat is effected by discharging onto the moving mat a mixture consisting of approximately ninety-five (95) per cent of pulverized quicklime, two (2) per cent of sodium chloride, and three (3) per cent of powdered sulphur, by weight, and then passing the mat having the said bleaching mixture intermixed therewith through warm water.

30 LOUIS D. JORDAIN.

REFERENCES CITED

The following references are of record in the file of this patent:

UNITED STATES PATENTS

| Number    | Name    | Date          |
|-----------|---------|---------------|
| 535,665   | Boyle   | Mar. 12, 1895 |
| 819,595   | Prins   | May 1, 1906   |
| 1,269,476 | Marsden | June 11, 1918 |
| 1,599,253 | Skolink | Sept. 7, 1926 |

OTHER REFERENCES

Paper Making Materials, by West, published 1928, by Lockwood Trade Journal Co., Inc., New York, N.Y., pages 173 and 174.